

Feb. 27, 1940.

J. E. CLEMENS ET AL

2,191,787

VOLTOLIZATION APPARATUS AND METHOD

Filed Dec. 17, 1936

2 Sheets-Sheet 1



John E. Clemens Inventor  
George L. Matheson  
By C. E. Young Attorney

Feb. 27, 1940.

J. E. CLEMENS ET AL

2,191,787

VOLTOLIZATION APPARATUS AND METHOD

Filed Dec. 17, 1936

2 Sheets-Sheet 2



John E. Clemens Inventor  
George L. Matheson Inventor  
By P. Young Attorney

## UNITED STATES PATENT OFFICE

2,191,787

## VOLTOLIZATION APPARATUS AND METHOD

John E. Clemens, Elizabeth, and George L. Matheson, Union, N. J., assignors to Standard Oil Development Company, a corporation of Delaware

Application December 17, 1936, Serial No. 116,256

9 Claims. (Cl. 204—31)

This invention deals with the voltolization of organic compounds and more specifically to a new method of voltolization as well as an apparatus therefor.

The term "voltolization" has been applied in recent years to the treatment of materials with silent electric discharges under vacuum. The process has been employed commercially for the thickening of mineral and fatty oils. In general the usual voltolization processes employ an alternating current of about 60-10,000 cycles a vacuum of 0.5 to 0.9 atmosphere and a voltage of 5,000-25,000 volts. The apparatus usually consists of a condenser type arrangement with the discharge taking place between two insulated electrodes, in which space is circulated a film of oil or other material to be treated. The latter is commercially achieved by the use of a rotating plate partially dipped in the charge stock, the upper part of the plate carrying the film subjected to the discharge.

One object of this invention is to obtain a higher degree of voltolization in a more efficient manner by the use of low voltage direct current. Another object is to carry out a discharge between uninsulated electrodes, one of which is in the form of a grid. Another object is to avoid the local overheating or deterioration of the feed stock (usually encountered due to "hot spots" when it is fed between electrodes) by placing the charge not between the electrodes but behind the cathode grid and allowing the discharge particles traveling through the grid electrode to impinge upon the feed stock. Further objects will be apparent from the subsequent disclosure.

The invention will be more clearly understood from the accompanying drawings in which Fig. 1 is a diagrammatic cross sectional elevation of a complete assembly of a voltolization apparatus operating on direct current. Fig. 2 illustrates a modified form of electrode assembly, while Fig. 3 is an electrode assembly suitable for operation with alternating current. Fig. 4 shows a front view of the grid and plate assembly.

Similar numerals refer to similar parts throughout the several views.

Numerals 1 designates a reaction shell or chamber capable of withstanding high vacuum. It is maintained by a suction pump evacuating at 2. In this chamber is located vessel 3 filled with oil 4 or oily organic compound or other raw material to be submitted to the electric discharge. Partially immersed in this oil is a rotating disc or plate 5, practically half the surface of which is in the oil bath. This plate is rotated by shaft

6 extending out of vessel 1 through packing gland 7, to driving gear 8 driven by motor 9. This shaft and reaction chamber are grounded at 10.

By rotating plate 5, an oil film 11 is formed on the surface subject to the action of the positive ions of the discharge, thereby causing a gradual thickening of the oil mass 4.

The discharge is produced as follows:

A positive electrode 12 which may be of any shape, such as wire, rod, tube, bar, grid, etc., is 10 led into chamber 1 through insulator 13. Opposite this electrode and as close to plate 5 as possible (without actual contact or wetting) is placed the negative electrode 14 which is in the form of a grid or foraminous plate having a 15 large amount of open space thereby allowing the positive ions 15 to pass therethrough and impinge upon the oil film 11 carried by plate 5. Grid electrode 14 is connected by means of conduit 16 to shaft 6 by sliding contact 17. It may be 20 suspended more rigidly from the top of chamber 1 by supports such as 18. With the connections shown, substantially no electrical potential gradient across the narrow space between grid electrode 14 and disc 5, the electrical potential in 25 disc 5 and electrode 14 tending to be equalized by their connection in common with conducting shaft 6.

A cooling coil 19 may be inserted in the oil reservoirs 3 so as to prevent overheating since 30 the ion impact on the grid 14 and oil film 11 raises the temperatures thereof.

Provision may also be made for bleeding in at valve 20 small amounts of various gases or vapors such as helium, argon, air, nitrogen, formaldehyde, hydrogen sulfide, sulfur dioxide, ammonia, etc.

It will be noted that in Fig. 1 only one side (11) of the rotating plate is subjected to the discharge. Fig. 2 illustrates a modification 40 whereby two grid electrodes and two positive electrodes may be arranged so as to voltolize the oil film on both sides of the rotating plate 5, the discharge zones being designated by 15. A multiple plate apparatus employing these principles is likewise possible.

The apparatus in Figs. 1 and 2 is designed for direct current operation. Although alternating current can be employed, only one-half of it will be utilized for thickening the oil, as can be seen 50 from the circuit. However, it is possible to obtain a higher efficiency with alternating current by employing the assembly shown in Fig. 3. The two plates 5 are insulated from each other by insulating member 21. An alternating current dis- 55

charge takes place between grids 14 intermittently from one grid to another as the polarity changes, and the positive ions passing through the grid impinge on the oil surface 11 carried by rotating 5 discs 5. The latter are connected with the electrodes by sliding contacts 22; hence the same electrical potential is impressed on each disc 5 at each instant as on its adjacent grid electrode 14, with which it is connected in parallel to an A. C. 10 power source, e. g., through a lead or bus bar 23. It will be noted that since only one phase voltolizes at a given instant, this method resembles the direct current procedure to that extent.

15 A front view of the grid and plate assembly is shown in Fig. 4. It will be seen that, since about one-half of the surface of the rotating plate 5 is immersed in oil bath 4 in reservoir 3, the grid 14 need be only semi-circular in shape fac- 20 ing the exposed oil film on plate 5.

The distance between the anode 12 and grid 14 may be any convenient distance, although it is preferable to maintain it at  $\frac{1}{2}$  to 2 inches. It is also preferable to construct grid 14 from Monel 25 metal, platinum, chrome steel (18% Cr and 8% Ni), nickel-chromium steels, etc., although Monel metal has been found highly satisfactory for this purpose.

Grid 14 should be placed as near oil film 11 30 as is practicable without wetting the grid, since the oil will carbonize on the surface, cutting off ion permeability. Of course, the ion impact on the grid tends to clean the grid surface to a great extent. As pointed out above, in order to 35 obtain the greatest amount of ion bombardment on the oil film 11, it is desirable to employ a grid having a maximum ratio of open space to metal area. It is also preferable to maintain as flat a grid surface as possible so as to obtain a more 40 even discharge from the anode.

Rotating plate 5 is preferably constructed of a conducting material such as aluminum, bronze, Monel metal, chrome steel, manganese-silicon bronze, etc. Since acids and other corrosive 45 compounds may be present, it is essential that a corrosion resistant material be employed so as to avoid contamination of the product. This plate has been observed to rise in temperature to about 150° F. after several days' operation. Where 50 such elevated temperatures are not desired, cooling may be resorted to, although sufficient cooling is effected by radiation, provided the current density is kept at about 10 to 30 milliamperes per square inch of plate surface.

55 By employing the apparatus disclosed in this invention it is possible to obtain excellent results with potentials of only about 300-600 volts. This, of course, depends to a great extent upon the apparatus, the pressure, and the inert gas 60 present. For instance, if hydrogen is present in chamber 1, a lower potential will be necessary to obtain the desired thickening action than if nitrogen were present.

In this type of apparatus, it is essential that 65 a low pressure be attained. It must be substantially below 10 mm. of mercury, say 5 mm. or 1 to 2 mm. or even a fraction thereof. In this respect the process differs considerably from other methods of voltolization which are preferably 70 carried out at 20 mm. or higher pressure.

Many advantages are gained by the type of voltolization described, herein. Due to the relatively low voltage employed, dielectric failures or difficulties are avoided. Since the type of dis- 75 charge is not affected to any appreciable extent

by the conductivity of the material treated, it is possible to voltolize highly polar compounds such as acids, bases, phenolic compounds and salts, which have been heretofore impossible to thicken in the usual condenser type discharge 5 wherein the charge stock is passed between the electrodes. Furthermore, it is even possible to voltolize solid or semi-solid materials by this means. This type of treatment is not limited to liquids or solids, but is likewise adapted for gase- 10 ous raw materials.

The temperature of voltolization is preferably kept at 50-150° F. although it is possible to carry out the treatment at temperatures as low as -100° F. or as high as 450° F. 15

The following examples illustrate the many phases involved in this invention:

#### Example 1

A sample of rapeseed oil having a viscosity at 20 100° F. of 250 seconds Saybolt and a viscosity of 56 at 210° F. was voltolized in an apparatus similar to that shown in Fig. 1 at 450 volts D. C., 10 milliamp per sq. in. current density, and 3 mm. Hg pressure for 8 hours. At the end of that period the viscosity of the oil was 130.7 at 210° F. and 25 869.5 at 100°. The current consumption was 13 kwh. per gal.

The product was an excellent blending agent 30 for lubricating oil.

#### Example 2

A mildly refined Pennsylvania oil of 150 viscosity at 210° F. was voltolized at 425 volts and 3 mm. Hg pressure with a current density of 15 35 milliamps per sq. in. in an apparatus similar to that shown in Fig. 1. At the end of 20 hours, the oil had a viscosity of 688 at 210° F. and proved to be an excellent lubricant as well as a blending agent for dispersing sludge in lubricating oils. 40 The current consumption was 40 kwh. per gal.

#### Example 3

Some stearophenone was voltolized as in Example 2 for 30 hours, and a thick product was obtained which in 2% concentration lowered the 45 pour point of the Pennsylvania oil by 20° F. The current consumption was 30 kwh. per gal.

#### Example 4

Rapeseed oil containing 8% sulfur was voltolized as in Example 2 for 7 hours, producing a thick oil which when blended in 10% concentration in an SAE 20 mineral lubricating oil, was able to carry all of the weights on the Almen machine without any bearing failure. The Almen 55 test dealing with extreme pressure lubrication is described in U. S. Patent 2,001,861.

This invention is not limited to any theory of operation or any specific examples, but only to the following claims in which the intention is to 60 cover the invention as broadly as the prior art permits.

We claim:

1. Method of voltolizing oily organic compounds which comprises projecting positive ions 65 from a gas ionizing zone through a narrow space having substantially no electrical potential gradient, then into contact with the organic compound in a liquid film at an interface of the film with said space, and exposing the surface of the 70 liquid oily organic compound film to the action of positive ions penetrating through said space until a desired substantial thickening of the organic compound is obtained.

2. Process of voltolizing liquid oily organic 75

- compounds which comprises setting up an electrical potential difference between opposite ends of a gas ionizing zone under conditions to produce positive gas ions projected toward a surface 5 of the liquid organic compound being treated, separating said surface of liquid compound being treated from said ionizing zone by a narrower zone across which substantially no electrical potential gradient exists but through which 10 positive ions produced in said ionizing zone are projected to impinge upon said surface of liquid compound being treated, and continuing the treatment of said liquid compound in this manner until a desired substantial thickening of the 15 organic compound is obtained.
3. Apparatus for thickening organic compounds, comprising a positive electrode, a grid-type negative electrode spaced from said positive electrode, electrical connections from said electrodes to complete an electrical circuit including 20 electrical potential difference between the positive electrode and the grid-type electrode to produce positive ions projected through openings in said grid-type electrode, and means electrically connected to have the electrical potential of the 25 grid-type electrode for exposing a liquid surface of the organic compounds to be thickened to bombardment by positive ions projected through openings in said grid-type electrode.
4. Apparatus for voltolizing an organic material comprising a plate adapted for rotation, means adapted to maintain on a surface of said plate a liquid film of the organic material having a gas-liquid interface, a grid-type cathode disposed parallel to said plate surface at a distance 30 to be just out of contact with a liquid film on said plate surface, a positive electrode situated about  $\frac{1}{2}$  to 2 inches from said grid-type cathode with the grid-type cathode interposed between said positive electrode and said plate; electrical connections from said positive electrode to a source of electric current, electrical connections from said grid-type cathode in an electric circuit for setting up an electrical potential difference between the grid-type cathode and the positive electrode so as to project positive ions emanating between said grid-type cathode and said positive electrode through 35
- openings in said grid-type cathode into contact with the liquid film at said gas-liquid interface, and electrical connections between said grid-type cathode and said plate for impressing substantially the same electrical potential on both 40 said grid-type cathode and said plate.
5. Apparatus for thickening an organic material comprising a pair of parallel plates electrically insulated from each other and adapted for rotation, means adapted to maintain liquid 45 films of the organic material on surfaces of said plates, a pair of parallel grid-type electrodes spaced apart between said pair of plates, each of said grid-type electrodes being disposed adjacent to one of said plate surfaces to be just beyond contact with a liquid film on its adjacent plate surface, means for connecting said grid-type electrodes to a source of alternating current for setting up electrical potential differences between said pair of grid-type electrodes so as to 50 project positive ions emanating between said grid-type electrodes alternately through openings in each of said grid-type electrodes to liquid films on their adjacent plate surfaces, and electrical connections from the source of alternating current to said plates for impressing the same voltage at each instant on each of said plates as is impressed on its adjacent grid-type electrode.
6. Process in accordance with claim 2 in which the potential difference between the opposite ends of said gas ionizing zone is from 300 to 600 volts. 55
7. Process in accordance with claim 2 in which the electric potential difference between the opposite ends of said gas ionizing zone is set up at a pressure below 10 millimeters of mercury.
8. Process in accordance with claim 2 in which the electric potential difference between the opposite ends of said gas ionizing zone is sufficient to maintain a current density of from 10 to 30 milliamperes per square inch.
9. Apparatus in accordance with claim 3 in which said means for exposing a surface of a liquid organic compounds to the action of positive ions is a plate adapted for rotation, the lower section of which is immersed in a reservoir containing said organic liquid compounds.

JOHN E. CLEMENS.

GEORGE L. MATHESON.